

## UNITED STATES PATENT OFFICE.

JOHN C. TATE, OF OAKLAND, CALIFORNIA.

## ABSORBING AND PURIFYING COMPOSITION.

No Drawing.

Application filed April 6, 1922. Serial No. 550,205.

*To all whom it may concern:*

Be it known that I, JOHN C. TATE, a citizen of the United States, and a resident of the city of Oakland, county of Alameda, 5 State of California, have made a new and useful invention—to wit, Improvements in Absorbing and Purifying Compositions; and I do hereby declare the following to be a full, clear, concise, and exact description 10 of the same.

The present invention relates to a modification of the absorbing and purifying composition described in my Letters Patent, granted July 13, 1920, under No. 1,346,349, 15 having the object of reducing the proportions and quantities and the combinations of the ingredients forming the composition.

This invention relates particularly to an absorbent composition or substance, consisting of either, the combination of mineral and vegetable matter, or a mineral substance and a binder, or a vegetable substance and a binder, or any one of the substances alone, which will absorb, wholly or in part, the 25 toxic parts of vitiated air or the injurious and objectionable gaseous products resulting from the combustion of hydrocarbon oils or gases.

A further object of the invention is to 30 provide a composition capable of retaining, absorbing and neutralizing moisture, gases and the disagreeable and injurious odors resulting from the combustion of animal and vegetable matter, permitting the combustion 35 of such matter in heating devices within restricted areas so as to not require outlets, flues or ventilation, usually necessary to the conventional type of gas or oil heater for carrying off the waste products of combustion. Other objects and advantages will 40 appear as this description progresses.

In this specification, the invention is described in the form considered to be the best, but it is to be understood that the invention 45 is not limited to such form, because it may be embodied in other forms; and it is also to be understood that in and by the claims following the description, it is desired to cover the invention in whatsoever form it 50 may be embodied.

The burning and combustion of hydrocarbon gases for heating and lighting, particularly the coal or water gas used in homes for illuminating and heating purposes, 55 leaves residuum exhaust gases which contain objectionable by-products unhealthful for

human inhalation and produce disagreeable odors, create moisture and tend to deface or attack metallic and painted surfaces and organic materials. 60

My invention contemplates an absorbent composition adapted to be contained within a suitable closure and to have the noxious exhaust gases (resulting from the combustion of hydrocarbons) to be passed through 65 and in contact with said composition. Carbon dioxid, sulfur gases, water vapor and the like, contained in the said exhaust gases, will thereby be absorbed or neutralized, such action resulting in the creation and libera- 70 tion of oxygen and the regeneration and purification of said exhaust gases into clean and wholesome air. In the practical operation of my invention, a heater or stove, utilizing hydrocarbon gases for combustion 75 purposes, would have a container mounted thereon and filled with lumps or particles of my absorbent composition. The exhaust gases from said burner would be passed through the container, into and with contact 80 with the absorbent composition and then discharged into the air to be heated. I have found by directing the course of the heated gases through the absorbent composition prior to releasing it into the atmosphere, 85

that the greater part of the toxic constituents of the exhaust gases are absorbed or neutralized, so that the heated air is released free of all noxious gaseous products and made fit for breathing purposes. The regeneration or purification of the heated gases in this manner eliminates the necessity of air vents to the said stove and makes it possible to do with gas heaters what has been commonly done with other heating appliances that do not generate objectionable gaseous products. The porous nature of the absorbent composition is such that it holds or retains the waste gaseous products, and repeated experiments have shown that the 90 absorbent composition is materially heavier after usage of a couple of months than when first placed in use, making it necessary to renew the composition only when saturated beyond a point of efficient absorption. 95

The composition is preferably formed of either a mineral absorbent, such as air-slaked lime, burned gypsum, kaolin or clay, either separately or mixed in combination with a vegetable absorbent, such as charcoal, 100 powdered dried corn cob or the like. The mineral absorbent (lime) may be used either

separately or mixed with a mineral binder and filler such as burned gypsum. A small quantity of clay or kaolin may be mixed directly with lime or included as an additional 5 element in combination with the lime and burned gypsum. Likewise, the mineral lime might be mixed directly with either wood charcoal or with the dried corncobs. Similarly, the vegetable absorbent, such as charcoal, 10 coal or the corncobs, might be mixed directly either with the mineral binder and filler, such as burned gypsum, or with clay or kaolin, in lieu thereof. The elements would be mixed in the following proportions, although it is to be understood that variations 15 in the quantities of said elements clearly come within the purview of this invention: lime, fourteen (14) to eighteen (18) parts; charcoal, one-half ( $\frac{1}{2}$ ) to two (2) parts; burned gypsum, six (6) to ten (10) parts; and kaolin, two (2) to six (6) parts. The 20 said approximate proportions would be adhered to when the ingredients would be used either separately or mixed in any of the combinations previously set forth.

The elements or ingredients would be preferably mixed in a dry powdered condition, to which water in a suitable quantity would be added to form a workable semi-solid mass. The mass would then be shaped or divided into units of any predetermined size and suitably dried. After being dried, the units are hard and porous. The lime of 30 the composition, which forms the greatest part thereof, acts as a retainer or absorber of water vapor and of the carbon dioxide and sulfur gases. The kaolin or clay acts in a similar manner and incidentally may be so treated as to act as a deodorant. The burned gypsum when used acts as a binder or filler 35 for holding all of the elements together and, furthermore, is porous and acts as a mechanical absorbent. The vegetable charcoal or corncob is likewise very dry and porous in body and it also serves as an absorbent 45 and neutralizer for reacting upon the gaseous products or impure air passed therethrough.

Having thus described this invention, what I claim and desire to secure by Letters Patent is:

1. A composition for purifying waste gaseous products of combustion comprising a vegetable material and a binder capable of absorbing and retaining moisture, gases 55 and the disagreeable odors resulting from the combustion of animal and vegetable matter.
2. A composition for purifying waste gaseous products of combustion comprising 60 charcoal and a binder capable of absorbing and retaining moisture, gases and the disagreeable odors resulting from the combustion of animal and vegetable matter.
3. A composition for purifying waste 65 gaseous products of combustion comprising a hard porous mass consisting of a mixture of charcoal and burned gypsum capable of absorbing and retaining moisture, gases and the disagreeable odors resulting from the 70 combustion of animal and vegetable matter.
4. A composition for purifying the waste 75 gaseous products of combustion comprising from one-half ( $\frac{1}{2}$ ) to two (2) parts by weight of wood charcoal and six (6) to ten (10) parts by weight of burned gypsum capable of absorbing and retaining moisture, gases and the disagreeable odors resulting from the combustion of animal and vegetable matter.

In testimony whereof, I have hereunto set my hand at San Francisco, California, this 28th day of March, 1922.

JOHN C. TATE.

In presence of—

LINCOLN V. JOHNSON.